

Nov. 12, 1929.

E. BACHE

1,735,030

METHOD FOR MAKING WATERPROOF PAPER BOARD

Filed Nov. 8, 1926



## UNITED STATES PATENT OFFICE

EDMUND BACHE, OF ST. PAUL, MINNESOTA, ASSIGNOR TO WALDORF PAPER PRODUCTS COMPANY, OF ST. PAUL, MINNESOTA, A CORPORATION OF MINNESOTA

## METHOD FOR MAKING WATERPROOF PAPER BOARD

Application filed November 8, 1928. Serial No. 146,963.

Heretofore, it has been attempted to render paper board impervious to moisture by impregnating an inner ply with asphalt or other waterproof material, or by applying a film of such material between the central or interior plies of the board. To adapt the product for use in constructing cartons and other paper board containers, it is necessary that the outer surfaces be porous or free from 10 waterproofing material other than the usual sizing. The waterproofing material has been applied either by mixing it with the stock supplied to one of the cylinders of a cylinder paper machine or by spraying or otherwise 15 spreading it upon an internal web or ply of the sheet during the passage of the web between successive cylinders. Unimpregnated webs or layers are then formed upon the waterproof layer during the passage of the web 20 over the succeeding cylinders of the machine, and the sheet is finally dried. Experience has taught that where a waterproofing agent in emulsified form, such as an emulsion of the soap type, is allowed to remain in the sheet, 25 this agent spreads to the surfaces, resulting in a staining or dyeing of the exterior by the emulsion. Such surface stains on the sheet render it unsuited for use in the construction of food containers and also interfere with 30 printing upon the surface and destroy the attractive appearance of the board.

It is the object of this invention to avoid such surface stains and to improve the waterproof qualities of the board by concentrating 35 the waterproof material in the interior thereof.

Briefly stated, my invention consists in applying an emulsion of a waterproof material, such as asphalt to the wet paper web 40 and then breaking down the emulsion, so that the asphalt particles coalesce in a natural state upon an interior web, after which the web continues through the machine and receives further layers of paper stock and is 45 finally passed through the dryer, where the heat spreads the asphalt particles, forming a continuous interior film. A suitable asphalt emulsion may be made from a natural asphalt blended with petroleum asphalt and 50 emulsified by a soap type of emulsifier.

About three per cent of sodium oleate and about forty per cent of water will form the desired emulsion with such asphalt. A suitable electrolyte for breaking down the emulsion may consist of a five per cent solution 55 of sulphuric acid, sprayed, or otherwise spread upon the emulsion.

The invention will be best understood by reference to the accompanying drawings, in which one form of my improved means are 60 shown attached to a cylinder paper machine of common type, the machine being illustrated diagrammatically. As here shown, the machine has six cylinders, indicated by the numerals 1 to 6 inclusive, adapted to form the 65 paper web from stock supplied to vats 7. A continuous blanket or felt 8 for supporting the paper web is passed over the upper periphery of the cylinders 1 to 6, inclusive, successively, and is held in contact therewith by 70 suitable couch rolls 9. As will be readily understood, the cylinders 1 to 6 apply successively layers of stock upon the felt 8. Between two of the cylinders, such as the cylinders 2 and 3, I provide a roller 10, adapted 75 to apply a suitable liquid waterproof material or emulsion thereof to the paper web formed by the cylinders 1 and 2. This roller 10 extends across the web in contact with the bottom surface thereof, and is revolved 80 within a small tank 11, adapted to be supplied with the waterproof material or emulsion through a pipe 12. Thus, a layer or film of waterproof material is applied to the web 85 as it passes over the roller 10.

The liquid waterproof material thus applied is now subjected to the action of an electrolyte which may be sprayed thereon from a supply pipe 13. The pipe 13 is extended transversely beneath the paper web 90 and is slotted or otherwise perforated along its upper periphery so as to spray the electrolyte upon the surface of the sheet previously supplied with the emulsion. The effect of the spraying of the emulsion with an electrolyte of positive nature is to break down the emulsion and cause the waterproof material to coalesce in its natural state upon the paper web. Now the web passes over the cylinders 95 3, 4, 5, and 6 successively where further 100

layers of stock are applied. Finally, the paper web is carried on in the usual manner between felt blankets to the dryers and, after drying, is delivered as a sheet having a 5 waterproof core and relatively pervious or porous surface plies. The heat of the dryers liquefies the asphalt in the interior layers and causes it to spread in a continuous film. In the finished sheet, the asphalt is concentrated 10 in the interior plies and is in its natural gummy state. It does not spread to the surfaces of the sheet during the drying as is the case when the more liquid or chemically active emulsions and particularly those of the 15 soap type are dried in the sheet.

It will be obvious that other methods of breaking down the emulsion may comprise impressing an electrostatic charge of positive nature upon the sheet, instead of applying 20 the electrolyte spray above described. Further, any suitable salt which will form an electrolyte of positive nature in an aqueous solution could also be used. Thus, aluminum sulphate, ferric chloride or calcium chloride 25 are suitable for forming the electrolyte spray in an aqueous solution. Nor is the present invention limited to the above described method of applying the emulsion to the sheet.

An important feature of this process is its 30 adaptability for use with emulsions containing an emulsifying agent of a chemically active type. Most emulsion of this type readily break down in the presence of dilute acids, and the emulsifying agents are at least 35 partially decomposed or oxidized upon the application of the heat of the dryers. Thus, the rectifying agent in no way detracts from the quality of the product, and it is even difficult to detect its presence in the sheet.

40 Having described my invention what I claim as new and desire to protect by Letters Patent is:

1. The method of making waterproof paper board which consists in first forming 45 an unimpregnated portion of the board, then applying to the interior surface of said portion an emulsified waterproof material without an admixture of fibrous stock, then breaking down the emulsion without the application 50 of heat to deposit the waterproof material upon the fibres in substantially natural state and subsequently drying the sheet.

55 2. The method of making waterproof paper board, which consists in applying to an interior portion thereof an asphalt emulsion containing an emulsifying agent of soap type, then applying to the film of asphalt 60 emulsion thus formed an electrolyte of positive nature adapted to cause the asphalt particles to coalesce upon the fibres and finally drying the sheet by the application of heat whereby the asphalt is spread in a substantially continuous film within the sheet,

and the emulsifying agent is at least partially decomposed.

3. The method of rendering paper board substantially impervious to moisture, which consists in first applying to a previously formed web an emulsion of a waterproof material of fusible nature, then breaking down said emulsion to cause said material to coalesce upon the fibres without the application of heat and finally spreading the coalesced waterproof material by the application of heat to the sheet to thereby form a substantially continuous layer of said material.

4. The method of rendering paper substantially impervious to moisture which consists in first forming a pervious portion of the sheet, then applying to an exposed surface of said portion an emulsified waterproof material of a fusible nature, then breaking down the emulsion without the application of heat to thereby cause said waterproof material to coalesce upon the fibres, then covering said waterproof material with pervious layers of stock and subsequently drying the sheet by the application of heat sufficient to liquefy and spread said material.

5. The method of rendering paper board substantially impervious to moisture, which consists in applying to a previously formed web emulsified waterproof material containing an emulsifying agent of chemically active type and without an admixture of fiber, then applying upon the exposed film of emulsion thus formed a dilute acid adapted to break down the emulsion and subsequently drying the sheet by the application of heat sufficient to at least partially decompose said emulsifying agent.

6. The method of making waterproof paper board which consists in first forming an unimpregnated portion of the board, then applying to the interior surface of said portion an emulsified waterproof material containing an emulsifying agent of chemically active nature, then breaking down the emulsion to deposit the waterproof material upon the fibres in substantially natural state and subsequently drying the sheet by the application of heat sufficient to at least partially decompose said emulsifying agent.

In testimony whereof, I have hereunto signed my name to this specification.

EDMUND BACHE.

120

125

130